

1

3,705,058

## SOFT-NITRIDING PROCEDURE FOR STEEL AND CAST IRON

Zoltan Kolozsvari and Endre Gal, Targu-Mures, Rumania, assignors to Fabrica de Utilaje si Piese de Schimb "Metalehnica," Targu-Mures, Rumania  
No Drawing. Filed July 7, 1971, Ser. No. 160,523  
Claims priority, application Rumania, July 9, 1970,  
63,864

Int. Cl. C23c 11/16, 11/18  
U.S. Cl. 148—16.6

1 Claim

### ABSTRACT OF THE DISCLOSURE

A method of increasing the nitrogen content of steel and cast iron wherein the body is maintained in an atmosphere of ammonia, methane and oxygen in a molar ratio of  $\text{CH}_4:\text{NH}_3=1$  and  $(\text{CH}_4+\text{NH}_3):\text{O}_2=25-30$  while maintaining the dissociation rate of the ammonia between 38 and 40%. The treatment time is 1 to 10 hours at a temperature of  $570^\circ\text{C.} \pm 10^\circ\text{C.}$

### SUMMARY

The invention refers to a soft-nitriding procedure of steel and cast iron in a controlled atmosphere, in order to increase the resistance of machine parts to scuffing, wear and fatigue.

The treatment has to be performed in a gaseous media composed of methane, ammonia and oxygen at a temperature of  $570 \pm 10^\circ\text{C.}$  The atmosphere has a high nitriding capacity and it is easy to control by common methods. The ratio of gas components is as follows:

$\text{NH}_3/\text{CH}_4=1$  and  $\text{NH}_3+\text{CH}_4/\text{O}_2=25-30$

As a result of the treatment a compound layer of a thickness of  $10-15 \mu\text{m.}$  is obtained, supported by a diffusion layer with a case depth depending on treating time and material composition.

The invention refers to a soft nitriding (low temperature carbonitriding) procedure of steel and cast iron in a controlled atmosphere.

Soft-nitriding of steel and cast iron machine parts is generally performed in a salt bath containing alkaline cyanides and cyanates. The active carbon and nitrogen appears as a result of decomposition of the above salts. The working temperature of the salt baths is of  $570 \pm 10^\circ\text{C.}$  (below of critical temperatures in Fe-N system). As result of the treatment a surface layer is to be obtained, composed of a compound (white) layer and a diffusion layer. The compound layer is responsible for the high resistance to wear and scuffing, the diffusion layer forms a support.

The above procedure presents disadvantages, because applying a salt bath with heavy toxic effect and by the other hand no continuous inspection and control of the bath characteristics is possible, the only inspection is by performing chemical analyses.

A soft-nitriding procedure in a gaseous media is also known, using Endo-gas and ammonia. Backdraw of this procedure is the use of gas generator and a low nitriding potential.

The procedure in conformity with the invention eliminates the above disadvantages, performing the nitriding in order to realize a controlled and uniform treatment, at  $570 \pm 10^\circ\text{C.}$  in an atmosphere composed of ammonia, methane and oxygen. The ratio of gas components is as

2

follows:  $\text{CH}_4/\text{NH}_3=1$  and  $(\text{CH}_4+\text{NH}_3):\text{O}_2=25-30$ , with an ammonia dissociation rate of 38-40%, and a treating time of 1-10 hours.

An example of realizing the invention is given below, in order to soft-nitride pieces of OLC 35 (plain carbon steel with 0.35% C).

The treatment has been performed in a gaseous media of the following composition:  $\text{NH}_3/\text{CH}_4=1$ , adding oxygen in a ratio of  $\text{CH}_4+\text{NH}_3/\text{O}_2=25-30$ , at a treating temperature of  $570 \pm 10^\circ\text{C.}$  The ammonia flow-rate has to be adjusted for a dissociation degree of 35-40%.

A three hours treatment assures the following results:

| Sample                     | Hardness |     |     |     |      |      |
|----------------------------|----------|-----|-----|-----|------|------|
|                            | HB       | HV1 | HV3 | HV5 | HV10 | HV30 |
| Untreated.....             | 200-207  |     |     |     |      |      |
| Nitrided in salt bath..... |          | 510 | 440 | 407 | 370  | 320  |
| Gas-nitrided.....          | 490      | 430 | 400 | 380 | 340  |      |

Metallographic examination has shown the following data:

case depth (of diffusion layer):  $0.35-0.40 \mu\text{m.}$

depth of compound layer:  $10-15 \mu\text{m.}$

microhardness of compound layer: 870-920 MHV.

On the basis of experiments the parameters of the above treatment, in conformity with the invention, have been established, as follows:

- (a) temperature:  $570 \pm 10^\circ\text{C.}$   
 (b) ratio of the components:  $\text{NH}_3/\text{CH}_4=1$  and  $(\text{CH}_4+\text{NH}_3):\text{O}_2=25-30$   
 (c) ammonia dissociation rate: 35-40%  
 (d) treating time can vary between 60 min. and 10 hours depending on parts to be treated and material.

Advantages of the procedure in conformity with the invention are:

a clean metal surface can be obtained  
 all the parameters of the procedure can be precisely checked and controlled.

What is claimed is:

1. A soft-nitriding procedure for increasing the nitrogen content of steel and cast iron articles, comprising heat treating said articles for 1 to 10 hours at a temperature of  $570^\circ\text{C.} \pm 10^\circ\text{C.}$  in an atmosphere of ammonia, methane and oxygen while maintaining the dissociation rate of the ammonia between 38 and 40%, said atmosphere being characterized by having molar ratios of  $\text{CH}_4$  to  $\text{NH}_3$  of 1 and  $\text{CH}_4+\text{NH}_3$  to  $\text{O}_2$  of 25 to 30.

### References Cited

#### UNITED STATES PATENTS

- 3,228,807 1/1966 Mitchell et al. .... 148—16.5 X  
 3,519,257 3/1968 Winter et al. .... 148—16.5 X  
 3,620,518 11/1971 Winter et al. .... 148—16  
 3,399,085 8/1968 Knechtel et al. .... 148—16.6

#### FOREIGN PATENTS

- 125,006 Czechoslovakia.  
 48,847 Germany.

65 CHARLES N. LOVELL, Primary Examiner

U.S. Cl. X.R.

148—16.5